

[54] **METHOD FOR THE DESULFURIZATION OF A STEEL MELT**

[75] Inventors: **Helmut Richter; Eckehard Forster; Edgar Spetzler; Jochen Wendorff, all of Oberhausen; Heinrich-Wilhelm Rommerswinkel, Mulheim, Ruhr, all of Germany**

[73] Assignee: **Thyssen Niederrhein AG Hutten-und-Walzwerke, Oberhausen, Germany**

[22] Filed: **Feb. 20, 1973**

[21] Appl. No.: **333,690**

[30] **Foreign Application Priority Data**

Mar. 1, 1973 Germany ..... 2209902

[52] **U.S. Cl. .... 75/58; 75/53**

[51] **Int. Cl. .... C21c 7/00**

[58] **Field of Search..... 75/58, 53**

[56]

**References Cited**

**UNITED STATES PATENTS**

|           |        |                 |       |
|-----------|--------|-----------------|-------|
| 3,268,326 | 8/1966 | Harders .....   | 75/58 |
| 3,575,695 | 4/1971 | Miyashita.....  | 75/58 |
| 3,598,573 | 8/1971 | Freissmuth..... | 75/58 |

*Primary Examiner*—P. D. Rosenberg

*Attorney, Agent, or Firm*—Karl F. Ross; Herbert Dubno

[57]

**ABSTRACT**

A steel melt is desulfurized in a ladle lined with dolomite magnesite or other refractory lining have an aluminum oxide content in excess of 70 percent (wt), by injecting at least 2,000 mm below the melt surface, finely divided calcium-containing compound after a basic-slag layer is applied to the surface of the deoxidized steel melt. The melt is held at a temperature of at least 1,530°C during desulfurization.

**11 Claims, 1 Drawing Figure**





## METHOD FOR THE DESULFURIZATION OF A STEEL MELT

### FIELD OF THE INVENTION

The present invention relates to a method of and to an apparatus for the desulfurization of a steel melt, and, more particularly, to the desulfurization of steel using calcium compounds.

### BACKGROUND OF THE INVENTION

In the treatment of steel melts, for example to eliminate clay-like particles which are suspended therein, it has been proposed to introduce calcium or a calcium compound in a finely divided form after an initial deoxidization of the melt, thereby achieving at the same time, the side effect of reduction of the sulfur content. However, this technique, in which the desulfurization is only a secondary reaction, has not proved to be effective in the reduction of the sulfur content to the degree needed in industry and hence the technique has not found widespread application as a desulfurization step when, for example, a sulfur content of 0.015 percent (wt) or greater in a steel melt is to be reduced to 0.005 percent (wt) or lower.

### OBJECTS OF THE INVENTION

It is the principal object of the present invention to provide an improved, economical and convenient method of reducing the sulfur content of a steel melt which allows a substantial reduction in the sulfur content so that, for example, a sulfur content of 0.015 percent (wt) of sulfur or greater can be reduced to 0.005 percent (wt) or less.

Another object of the invention is to provide a method of desulfurizing a steel melt which is relatively efficient, avoids disadvantages hitherto encountered in the desulfurization of steel, and can be carried out with convenient and economical apparatus.

Still another object of the invention is to provide a process and apparatus for the desulfurization of steel which yields a product of convenient composition, without disadvantages hitherto encountered with desulfurization techniques.

### SUMMARY OF THE INVENTION

It has now been found, most surprisingly in light of previous experience with the introduction of calcium-containing compounds into a steel melt, that reductions of the sulfur level in a steel melt containing 0.015 percent (wt) sulfur to a level of 0.005 percent (wt) or less can be achieved by controlling certain critical parameters of the system for introducing the calcium-containing substances and by protecting the surface of the melt into which the calcium-containing substances are injected with a particular slag composition. More particularly, it has been found that, when the melt is initially deoxidized and then covered by a basic-slag layer containing at most 4 percent (wt) FeO, and the calcium-containing substances are injected in finely divided form at least 2,000 mm below the surface of the slag-covered melt in a neutral carrier gas, the desulfurization obtainable is far and above any which could have been predicted from knowledge of the secondary reaction or side effect mentioned earlier. In fact, desulfurization to sulfur contents substantially less than 0.005 percent (wt) are obtainable in this manner and

a sulfur content of 0.015 percent (wt) can be brought to this level (i.e., 0.005 percent by weight).

The present invention thus resides in a method of desulfurizing a steel melt which comprises the steps of deoxidizing the steel melt by adding thereto a deoxidizing agent, such as aluminum, in accordance with conventional practice. Since the deoxidation step is conventional in the art and can be carried out by any of the techniques known therein without affecting the present invention, there is no need for a special discussion of the deoxidization step. Suffice it to say that, subsequent to deoxidization, the steel melt according to the present invention is covered with a basis slag containing less than 4 percent (wt) FeO and preferably less than 2 percent (wt) FeO, the slag layer having a thickness sufficient to prevent dislocation of the slag layer is not critical although this thickness may range from 20 mm to 100 mm without affecting the operation of the system of the present invention in any way. Preferably 2 to 15 kg of slag is used per ton (metric) of the deoxidized steel melt.

According to the present invention, the desulfurized steel melt, covered immediately after deoxidization with a basic-slag layer having an FeO content of less than 4 percent (wt) at a temperature above the boiling point of calcium (1,490°C) and preferably at least 1,530°C is treated with a stream of calcium (elemental), a calcium alloy, an intermetallic calcium compound or an ordinary calcium compound (collectively referred to hereinafter as calcium-containing substance) in a carrier gas stream by injection thereof at least 2,000 mm below the surface of the melt. Advantageously the calcium-containing substance may include atoms of an element (e.g., carbon, nitrogen, silicon) the proportion of which is to be increased in the melt.

When a basic slag has an FeO content in excess of 2 percent (wt), it is preferred in accordance with the present invention to maintain the blowing operation in which a calcium-containing substance in finely divided form is injected into the melt in the carrier gas, until the FeO concentration in the slag falls to or below 2 percent (wt). Advantageously, the slag alone may be blown until the FeO content is less than 2 percent (wt) using a lance through which the calcium-containing substance in the inert or neutral carrier gas is introduced, whereupon the lance is plunged below the surface of the melt to a depth of at least 2,000 mm to carry out the injection of the calcium-containing substance, the overlying slag having thereby had its FeO content reduced.

Substantially any carrier gas which does not enter into reactions with the melt and the calcium-containing substance may be employed, although the inert gases such as argon are preferred. The calcium-containing substance may be elemental calcium, as noted above, calcium-silicon intermetallic compounds or alloys, or calcium carbide. Preferably the calcium-containing substance has a boiling point or thermal decomposition point below 1,530°C. When the term "finely divided" is used herein, it is intended to refer to solids of a particle size such that they are readily entrainable in the gas stream at the pressure required to inject the gas and solids at least 2,000 mm below the surface of the melt. The particle size may range from the order of microns to several millimeters. Preferably the calcium-containing substance is introduced in an amount corresponding to 1.2 to 1.5 kg of calcium per ton of the melt.

In order to appreciate the differences between the injection process, as described above, and the art in which calcium introduction into a steel melt results in desulfurization as a side reaction, it should be noted that oxygen from the slag used in these latter systems returns to the steel melt during the process and the slag permits a transfer of calcium sulfide from the slag to the melt. With the basic slag of the present invention, having a low FeO content, this cannot occur.

According to a more specific feature of this invention, the slag contains: 45 to 75 percent (wt) calcium oxide (CaO), and preferably 45 percent to 55 percent with best results at about 50 percent (wt) CaO, between 0 and 25 percent (wt) calcium fluoride (CaF<sub>2</sub>) and preferably about 20 percent (wt) of the CaF<sub>2</sub>, 0 to 20 percent (wt) aluminum oxide (Al<sub>2</sub>O<sub>3</sub>) and preferably 10 to 20 percent with best results at about 12 percent (wt) Al<sub>2</sub>O<sub>3</sub>, 0 to 30 percent (wt) silicon dioxide (SiO<sub>2</sub>), preferably 5 to 30 percent with results of about 10 percent (wt) SiO<sub>2</sub>, 0 to 4 percent (wt) FeO and preferably 0.5 to 1 percent (wt) FeO, 0 to 10 percent (wt) manganese oxide (MnO), phosphorus pentoxide (P<sub>2</sub>O<sub>5</sub>) and magnesium oxide (MgO), each, with up to 10 percent (wt) of all of these latter compounds and preferably no more than 7.5 percent (wt) thereof, taken together.

A preferred slag composition is: 50 percent (wt) CaO, 20 percent (wt) CaF<sub>2</sub>, 12 percent (wt) Al<sub>2</sub>O<sub>3</sub>, 10 to 20 percent (wt) SiO<sub>2</sub>, 0.5 to 1 percent (wt) FeO, up to 7.5 percent (wt) phosphorus pentoxide, magnesium oxide and manganese oxide.

Tests have shown that the minimum depth of injection of the calcium-containing substance of 2,000 mm is critical and that attempts to reduce this depth, with or without the use of a slag layer, results in desulfurization which is not sufficient from a technological and economical point of view. Furthermore, the minimum temperature must be 1,490°C, although, for practical considerations, a temperature of 1,530°C is the minimum. Of course, when the calcium-containing substance has a higher melting point or dissociation point, the latter temperature is the minimum.

The melt is a steel melt which is treated after oxidation and should not be confused with a pig iron or other melt which is to be converted to steel. The desulfurized steel melt which is employed, according to the invention, should have a residual deoxidizer concentration of 0.015 percent (wt) or greater at the time the calcium particles are injected. It is indeed surprising that the presence of residual deoxidizer in the melt increases the efficiency of the desulfurizing operation since one normally would expect that the high affinity of calcium for oxygen would render superfluous any residual deoxidizer.

According to another feature of the invention, the steel melt is treated in a ladle lined with dolomite, magnesite or some other refractory composition having a high aluminum oxide content, i.e., an aluminum oxide content of at least 70 percent (wt). This contrasts with the fire clay linings normally used on deoxidization ladles and has been found to be advantageous in blocking oxygen penetration to the melt and in increasing the degree to which the melt can be desulfurized using the injection of calcium-containing substance as previously described. The ladle is preferably provided with a slide-type closure rather than a stopper lined with fine clay.

## DESCRIPTION OF THE DRAWING

The above and other objects, features and advantages of the invention will become more readily apparent hereinafter, reference being made to the accompanying drawing in which the sole FIGURE is a diagrammatic vertical section through a desulfurization ladle for carrying out the method of the invention.

## SPECIFIC DESCRIPTION

The drawing shows a ladle 10 for the desulfurization of a previously deoxidized steel melt 11 which comprises a steel vessel 12 having a lining 13 of dolomite, magnesite or mixtures thereof with one another and having an aluminum oxide content of at least 70 percent (wt) Al<sub>2</sub>O<sub>3</sub>. Instead of the stopper normally used with such ladles, the discharge spigot 14 thereof is closed by a slide plate 15.

Above the deoxidized steel melt 11, there is provided a layer of basic slag 16 through which a lance 17 reaches to a location which lies at a distance D of at least 2,000 mm below the level of the bath.

The lance is supplied with argon from a source 18 and with a calcium-containing substance in finely divided form from a metering device 19.

As pointed out earlier, the steel melt is deoxidized (e.g., by the addition of aluminum to the melt 11) in the ladle 10, until the aluminum content of the steel is stable at about 0.015 percent (wt), thereby indicating that deoxidization is complete. The basic slag is thereupon immediately applied to the melt and, if the basic slag has an FeO content in excess of 2 percent (wt), the calcium-containing substance is injected until the FeO level drops below 2 percent (wt). The lance is then plunged to a depth of 2,000 mm or more and blowing is continued until the desired degree of desulfurization is achieved.

## SPECIFIC EXAMPLE

A fireclay-lined ladle having a depth of 4.00 m is charged with 120 tons of molten steel which is deoxidized until the steel has essentially the following composition: 0.15 percent (wt) carbon, 0.10 percent (wt) silicon, 0.50 percent (wt) manganese, 0.070 percent (wt) phosphorus, 0.006 percent (wt) nitrogen, 0.015 percent (wt) sulfur, 0.045 percent (wt) metallic aluminum, the balance being Fe. 6.5 kg of a slag, per ton of molten steel, is then supplied, the slag having substantially the following composition: about 50 percent (wt) CaO, about 20 percent (wt) CaF<sub>2</sub>, about 12 percent (wt) Al<sub>2</sub>O<sub>3</sub> about 10 percent (wt) SiO<sub>2</sub>, about 0.5 percent (wt) FeO, the balance being manganese oxide, phosphorus pentoxide and magnesium oxide.

The melt was blown by a lance inserted to a depth of 2.60 m below the level of the steel bath with a calcium-silicon alloy (calcium ferrosilicon) containing 30 percent (wt) calcium, 60 percent (wt) silicon, 10 percent (wt) Fe at a rate of 4.4 kg of the calcium-containing substance per ton of molten steel. The carrier gas was argon. The calcium-silicon substance had a particle size between 25 and 150 microns. After blowing, the steel has the following composition: 0.15 percent (wt) carbon, 0.37 percent (wt) silicon, 0.50 percent (wt) manganese, 0.10 percent (wt) phosphorus, 0.006 percent (wt) nitrogen, 0.017 percent (wt) metallic aluminum, 0.005 percent (wt) sulfur, balance iron.

The calcium utilization, calculated in terms of CaS, is about 10 percent. When the metallic aluminum is present in the steel melt in an amount of 0.040 percent (wt), but the lining is changed to have an aluminum oxide content of 70 percent (wt) the sulfur concentration can be reduced to 0.004 percent (wt) or less. The best results are found with aluminum levels in excess of 0.020 (wt).

Similar results are obtained when elemental calcium is introduced except that the silicon content remains unaltered. When it is desired to increase the carbon content, calcium carbide is used in the same proportions. The slag composition may be varied wide ranges as noted above and it is preferred to provide a slag containing at least 50 percent calcium oxide and up to 75 percent thereof. A synthetic slag may be formed by depositing 75 percent (wt) calcium oxide and 25 percent (wt) calcium fluoride on the top of the deoxidized steel melt.

We claim:

1. A method of desulfurizing a deoxidized steel melt, comprising the steps of:

covering the deoxidized steel melt with a basic-slag layer containing at most 4 percent by weight FeO; introducing at a location at least 2,000 mm below the surface of the deoxidized steel melt covered with said basic slag layer a stream of a calcium-containing substance in finely divided form in a neutral carrier gas;

maintaining the temperature of said melt during the introduction of said calcium-containing substance thereto at at least 1,530°C,

maintaining said molten steel in contact with a lining containing at least 70 percent by weight aluminum oxide during introduction of the calcium-containing substance thereto; and

the introduction of said calcium-containing substance is carried out so that said steel melt contains at least 0.015 percent by weight aluminum.

2. The method defined in claim 1 wherein said basic-slag layer has an FeO content in excess of 2 percent, further comprising controlling the introduction of the calcium-containing substance to reduce the FeO content of the basic slag layer to less than 2 percent by

weight.

3. The method defined in claim 1 wherein said gas is argon.

4. The method defined in claim 3 wherein said calcium-containing substance is introduced into said melt by a lance extending downwardly through the melt.

5. The method defined in claim 1 wherein said basic slag layer has essentially the following composition: 45 to 75 percent by weight calcium oxide, 0 to 25 percent by weight calcium fluoride, 0 to 20 percent by weight aluminum oxide, 0 to 30 percent by weight silicon oxide, 0.1 to 4 percent by weight FeO, and 0 to 10 percent by weight manganese oxide and/or phosphorus pentoxide and/or magnesium oxide.

15 6. The method defined in claim 5 wherein said slag has approximately the following composition: 50 percent by weight calcium oxide, 20 percent by weight calcium fluoride, 12 percent by weight aluminum oxide, 10 percent by weight silicon oxide, 0.5 percent by weight FeO, the balance being manganese oxide, phosphorus pentoxide and magnesium oxide.

7. The method defined in claim 5 wherein said calcium-containing substance is added to said melt in an amount corresponding to substantially 1.2 to 1.5 kg of calcium per ton of molten steel.

8. The method defined in claim 7 wherein said calcium-containing substance is selected from the group which consists of elemental calcium, a calcium-silicon, intermetallic compound or alloy, and calcium carbide.

9. The method defined in claim 8 wherein said calcium-containing substance is a calcium ferrosilicon containing substantially 30 percent by weight calcium, 60 percent by weight silicone and 10 percent by weight iron, the calcium ferro silicone being introduced into said melt in an amount of substantially 4 to 5 kgs per ton of molten steel.

10. The method defined in claim 8 wherein said molten steel contains at least 0.015 percent by weight of the deoxidizing agent for said melt.

11. The method defined in claim 1 wherein said slag layer is present in an amount of substantially 1 to 15 kgs per ton of molten steel.

\* \* \* \* \*

**REEXAMINATION CERTIFICATE (598th)**  
**United States Patent [19]** [11] **B1 3,885,957**  
**Richter et al.** [45] **Certificate Issued Dec. 16, 1986**

[54] **METHOD FOR THE DESULFURIZATION OF A STEEL MELT**

[75] **Inventors:** Helmut Richter; Eckehard Forster; Edgar Spetzler; Jochen Wendorff, all of Oberhausen; Heinrich-Wilhelm Rommerswinkel, Mulheim, all of Fed. Rep. of Germany

[73] **Assignee:** Thyssen Niederrhein AG  
Hutten-und-Walzwerke, Oberhausen,  
Fed. Rep. of Germany

**Reexamination Request:**

No. 90/000,905, Nov. 15, 1985

**Reexamination Certificate for:**

Patent No.: 3,885,957  
Issued: May 27, 1975  
Appl. No.: 333,690  
Filed: Feb. 20, 1973

[30] **Foreign Application Priority Data**

Mar. 1, 1973 [DE] Fed. Rep. of Germany ..... 2209902

[51] **Int. Cl.<sup>4</sup>** ..... C21C 7/00

[52] **U.S. Cl.** ..... 75/58; 75/53

[58] **Field of Search** ..... 75/53, 58

[56] **References Cited**

**U.S. PATENT DOCUMENTS**

|           |         |                  |       |
|-----------|---------|------------------|-------|
| 2,577,764 | 12/1951 | Hulme            | 75/51 |
| 2,992,097 | 7/1961  | Spence           | 75/55 |
| 3,192,037 | 6/1965  | Haucke et al.    | 75/55 |
| 3,575,695 | 4/1971  | Miyashita et al. | 75/51 |
| 4,392,887 | 7/1983  | Goedert          | 75/53 |

**FOREIGN PATENT DOCUMENTS**

|         |         |                      |   |
|---------|---------|----------------------|---|
| 183097  | 9/1955  | Austria              | . |
| 207395  | 1/1960  | Austria              | . |
| 1408188 | 10/1968 | Fed. Rep. of Germany | . |
| 4626612 | of 1971 | Japan                | . |
| 818697  | 8/1959  | United Kingdom       | . |
| 829274  | 3/1960  | United Kingdom       | . |

**OTHER PUBLICATIONS**

*Journal of the Iron and Steel Institute*, Jun. 1960, Desulphurization of Basic Arc Furnace Steel by the Injection of Powdered Materials, pp. 195-201, L. Marples, B.Sc., A.R.I.C., and J. Pears, Assoc. Met., A.I.M.

*Neue Hütte*, 16, 2, 72-7 (Feb. 1971), A New Method of Desulfurizing Steel, Nils F. Grevillius, Lars-Erik Carlsson, and Lars Hellner Bofors (Sweden) (with English language translation).

*Stainless Steel Making*, *Iron and Coal*, Sep. 4, 1961, pp. 461-462.

H. J. Langhammer and D. Danckert, Bremen, "Comparison of Processes for Continuous and Discontinuous Desulphurization with Different Desulphurizing Agents", *Radex-Rundschau*, Journal 1, 1971, pp. 3-25. Kiichi Narita, Akitsu Tomita, Yasuo Hirooka and Yoshitomo Satoh, "Desulphurization of Molten Pig Iron

by Means of Injection Method", 56, 1970, pp. 1602-1612.

*Stahl und Eisen*, 91, 1971, No. 3, *Umschau*, pp. 151-154 (with English translation).

Leitner-Plockinger, "Production of Special Steel", *Edelstahlerzeugung*, 1965, pp. 209-210, 555, 681-682 (with English translation).

Helmut Knuppel, "Desoxydation und Vakuumbehandlung von Stahlschmelzen", 1970, pp. 62, 69, 275-283 (with English translation).

"Die Physikalische Chemie der Eisen- und Stahlerzeugung", 1964, pp. 259-261, 329 (with English translation).

Bernhard Osann, "Lehrbuch der Eisenhuttenkunde", 1921, pp. 540-545, (with English translation).

Bernhard Osann, "Die Entschwefelung des FluBeisens im elektrischen Induktionsofen", *Stahl und Eisen*, Jul. 15, 1908, pp. 1017-1022, (with English translation).

*Iron & Steel*, p. 85, No. 3, vol. 55 (1969).

*Handbook of Iron and Steel*, Fig. 8.125 in p. 668, printed by Maruzen (Mar. 1971).

Manufacture of Cast Iron and Steel, Table 10.4 in p. 458, printed by Yohkendo.

*Iron & Steel*, pp. 998-1013, No. 8, vol. 56 (1970) (with English translation).

"Progress in Processes for Melting Steel Under Vacuum and for Degasifying under Vacuum", pp. 147-157, "RH Degasifying Method", printed by Japanese Iron and Steel Association (1969).

Edward J. Dunn, Jr., "Rapid Desulfurization to 0.002 Percent Sulfur", *Modern Castings*, pp. 90-95, No. 6 (1961).

George J. McManus, "It's What's in the Ladle that Counts in Refining", *Iron Age*, May 7, 1979, pp. 11-14.

33 Metal Producing, Apr. 1981, "Ladle Injection Metallurgy: where it's at, where it's going, and why", pp. 53-59.

Harold E. McGannon, "The Making, Shaping and Treating of Steel", Ninth edition, pp. 38 and 64.

English language translation of the decision of the Federal Patent Court of the Federal Republic of Germany, Dec. 19, 1979.

S. Santen and B. Ohman, "Techniques for Obtaining Extremely Low Contents of Sulfur in Steel Under Oxidizing and Reducing Conditions", Swedish Academy of Engineering Science, Stockholm 1971, Report 196-1, pp. 7-19.

**Primary Examiner—P. D. Rosenberg**

[57] **ABSTRACT**

A steel melt is desulfurized in a ladle lined with dolomite magnesite or other refractory lining have an aluminum oxide content in excess of 70 percent (wt), by injecting at least 2,000 mm below the melt surface, finely divided calcium-containing compound after a basic-slag layer is applied to the surface of the deoxidized steel melt. The melt is held at a temperature of at least 1,530° C. during desulfurization.

**REEXAMINATION CERTIFICATE  
ISSUED UNDER 35 U.S.C. 307**

THE PATENT IS HEREBY AMENDED AS  
INDICATED BELOW.

Matter enclosed in heavy brackets [ ] appeared in the  
patent, but has been deleted and is no longer a part of the  
patent; matter printed in italics indicates additions made  
to the patent.

The drawing figure has been changed as follows:  
"Dolomite/Magnesite" has been deleted before "lin-  
ing".

**5 AS A RESULT OF REEXAMINATION, IT HAS  
BEEN DETERMINED THAT:**

The patentability of claims 1-11 is confirmed.

10 New claim 12 is added and determined to be patent-  
able.

12. *A method according to claim 1, wherein said steel is  
desulfurized to a sulfur level of at least 0.005 weight per-  
cent.*

\* \* \* \* \*

20

25

30

35

40

45

50

55

60

65